

## UNITED STATES PATENT OFFICE

1,950,471

## MANUFACTURE OF CREPE YARNS

Eduard Boos, Oberbruch, Kreis Heinsberg, Germany, assignor to American Glanzstoff Corporation, New York, N. Y., a corporation of Delaware

No Drawing. Application March 1, 1932, Serial No. 596,162. In Germany March 24, 1931

2 Claims. (Cl. 28—1)

My present invention concerns the production of crepe yarn from artificial filaments.

One object of the invention is to provide a novel, yet simple, method for the production of 5 crepe yarn.

Other objects will become apparent from a consideration of the following specification.

According to one process by which I produce 10 a crepe effect on artificial filaments, specifically artificial viscose filaments, the filaments are extruded in the regular manner. They are then after-treated but are maintained in an undesulphurized state. Because the sulphur has not been removed it adheres to the filaments 15 throughout their manufacture, and when these undesulphurized filaments are made up into a yarn, the sulphur acts as a sizing agent.

After the production of the yarn itself, the 20 fabric may be finished by treatment with diluted lyes which act to shrink the undesulphurized portions of the yarn, at the same time removing the sulphur therefrom. I have found that undesulphurized yarns possess noted shrinking tendencies and thus the production of a crepe effect 25 yarn is facilitated.

According to another process whereby I produce crepe effect yarn, I make use of untwisted 30 artificial filaments. Ordinarily, when twisted filaments are to be used in the manufacture of crepe yarn, it is necessary to supply certain of the filaments with a decided left-hand twist. When using yarn which has been twisted, this 35 twist must be compensated for when the crepe-making twist is applied. I overcome this difficulty by leaving the original silk untwisted and collecting it, as it is newly spun, directly upon the usual cylinders, spools or reels. This 40 untwisted yarn while upon these holders may be suitably washed and dried. It may then be run directly upon twisting spools, and the proper left- or right-hand twist applied, whereupon it 45 may be used in the manufacture of crepe effect yarn. By "proper" it is meant that the thread or yarn is twisted to a high degree, i. e., to that 50 degree necessary to give the "proper" or "high" twist necessary to produce crepe yarn. It will be noted that the absence of the ordinary twist in the present case does away with the necessity of compensating for this twist, or possibly 55 of untwisting the yarn, which expedients are necessary when the ordinary process is used. In making filaments of this type they are allowed to remain in the undesulphurized state, as I have found that the sulphur acts as a binding

or sizing agent and enables the handling of the filaments while they are thus untwisted.

In the event that this present process is to be used in connection with the production of viscose filaments according to the spool spinning process, it has been found that several steps will be eliminated from the usual process and thus danger of damaging the artificial filaments by handling is decreased. Spool yarn is that which is wound, after production, directly upon a spool. 60 While upon this spool, which may be perforated, for example, the yarn is after-treated without any intermediate rewinds. According to my present process, I lay the untwisted yarn directly upon the spools, treat it by washing, but do not 65 desulphurize it. Thus, as is pointed out above, the sulphur remains in the filaments to act as a sort of a binder or sizing and enables the filaments to be handled in their untwisted state.

The sulphur may be removed from the crepe 70 yarn without any difficulty after it has been woven. After the desulphurization of the woven yarn occurs, the shrinkage of the filaments is occasioned, and the desired crepe effect is produced.

Having now set forth my invention as required by the statutes of the United States Patent Office, what I desire to claim is:

1. In the manufacture of crepe effect fabrics, the steps of producing viscose filaments, winding them while untwisted upon spools, washing the untwisted filaments without desulphurizing, applying high left- and right-hand twists to the filaments thus produced, making them up into a fabric, and then desulphurizing the resulting 85 fabric.

2. In the manufacture of crepe effect fabrics, the steps of producing viscose filaments, winding them while untwisted upon spools, washing the untwisted filaments without desulphurizing, 90 applying high left- and right-hand twists to the filaments thus produced, making them up into a fabric, and then desulphurizing the resulting 95 fabric through the use of a dilute caustic solution.

EDUARD BOOS.

100

105

110